

July 7, 1936.

G. SIGLER

2,046,347

METHOD OF MAKING ARTIFICIAL THREAD

Filed Dec. 15, 1933

2 Sheets-Sheet 1

Fig. 1.



INVENTOR

George Sigler

BY

Wm S. Pitchard

ATTORNEY

July 7, 1936.

G. SIGLER

2,046,347

METHOD OF MAKING ARTIFICIAL THREAD

Filed Dec. 15, 1933

2 Sheets-Sheet 2

Fig. 2.



INVENTOR  
George Sigler  
BY  
Wm S. Pitchard  
ATTORNEY

## UNITED STATES PATENT OFFICE

2,046,347

## METHOD OF MAKING ARTIFICIAL THREAD

George Sigler, Richmond, Va., assignor to Du Pont Rayon Company, New York, N. Y., a corporation of Delaware

Application December 15, 1933, Serial No. 702,537

5 Claims. (Cl. 18—54)

This invention relates to the manufacture of artificial threads, filaments or the like. More particularly, the invention relates to the production of artificial threads having substantially uniform shrinkage characteristics.

One of the methods of preparing regenerated cellulose threads comprises spinning a viscose solution and, after regeneration of the cellulose, collecting the newly formed thread on a rotating bobbin, commonly termed the "spin bobbin", where it is laid down in the form of a cake by means of a traversing mechanism. The thread normally consists of a ribbon-like bundle of parallel filaments which is subsequently washed acid-free by any one of a number of procedures, such as, for example, by forcing water outwardly through the cake. The washed thread, according to the usual practice, is then dried on the spin bobbin and the dried thread is thrown to another bobbin or spool by means of a throwing machine, whereby the thread is twisted to the desired number of turns per inch. Alternatively, the dried thread is spooled and the spooled yarn twisted in the manner mentioned. The dried, twisted thread is then reeled into skeins and the latter are subjected to the purifying operations, i. e., desulphuring and bleaching. In some instances the dried, twisted thread on the second bobbin is subjected to the purifying operations.

It is a well-known fact that rayon thread shrinks during the drying operation. If, during the initial drying step, the thread is freely suspended, it will shrink at least 5% of its original length and indeed as much as 10% of its original length. However, since in the methods above mentioned the rayon thread is dried against a rigid support, i. e. a spin bobbin, much of the shrinkage is prevented and prevented non-uniformly. As a consequence, the thread, when again wetted and dried in the subsequent operations, additionally shrinks non-uniformly.

The unevenness of the shrinkage in terms of residual shrinkage throughout a bobbin cake of yarn, when it is dried by the usual method on a rigid body, can be readily illustrated by plotting a curve with % shrinkage as abscissa and length through the cake as ordinates. Residual shrinkage is explained as follows:

A package of yarn is reeled into 1,000 yard skeins; the skeins are measured, showered for 60 minutes with 1.35% caustic solution at 95° C., washed free from caustic with soft water and then dried in a freely suspended condition. The length of the skeins is measured and the per-

centage difference between the original and final lengths is termed the "residual shrinkage".

Upon reference to a curve plotted as above described it will be noted that the yarn comprising the middle portion of the cake is shrunk to a considerably larger extent, i. e. has less residual shrinkage than either the innermost or outermost parts of the cake, so that the residual shrinkage of yarn varies about 4% from maximum to minimum or, in other words, the minimum is less than one-half the maximum. This variation in shrinkage is highly objectionable, because skeins wound therefrom and subjected to the customary desulphuring and bleaching operations shrink unevenly. Such yarn, when back-wound, produces an excessive number of stops and breaks, resulting in a large number of broken filaments, an excessive amount of fluff and, in general, lower quality yarn. This non-uniformity of shrinkage is indicative of uneven dyeing characteristics throughout the cake, and it has been found that the affinity for direct dyes is sufficiently diminished by the tension built up during drying to render the yarn unsuitable for its intended purpose.

If in any process wherein the thread is dried in the presence of a rigid support, as on the spin bobbin, the yarn is subsequently reeled into skeins, wetted and dried freely, the non-uniformity of shrinkage is overcome but only at a great sacrifice to the quality of the resultant skein. A skein produced as just mentioned is customarily referred to as a tight and loose skein. It is extremely difficult to handle, because that part of the skein containing thread which has a high residual shrinkage shrinks to a considerably greater extent than that part of the skein which contains lower residual shrinkage thread. This uneven shrinkage means that the loops of thread comprising the skein may be different in diameter by one-half inch or more. When such a skein is placed on a swift for unwinding, the tight loops are stretched while the loose loops are slack and tend to tangle and knot as the skein is unwound. Furthermore, in the normal reeling process, if the skein reeled is from the inside of the spin cake, the portion comprising the inner winding of the skein (the cake has been reversed in throwing) is that part which will shrink most and become tight thread.

I have found that the above-mentioned defects and disadvantages can be overcome and artificial thread having substantially uniform shrinkage characteristics can be obtained by

twisting gel thread from a package and winding the twisted thread on to a take-up device in a substantially dry or semi-dry condition, the twisting and winding operations being successive and continuous, and thereafter converting into skeins and purifying. Specifically, I have found that the desired results can be secured by twisting acid free gel thread, by the throwing of the same prior to skeining and purifying. In the throwing operation, I have found that during the ballooning of the thread a drying is effected in a convenient space.

It is, therefore, an object of this invention to prepare bobbin spun rayon of substantially uniform shrinkage characteristics.

A still further object is to produce a bobbin spun rayon of improved dyeing characteristics.

Another object of this invention is to produce bobbin spun rayon of superior textile properties and which is free from factors responsible for low quality.

A specific object of this invention is to provide a method of twisting gel rayon and winding the thread in a dry or semi-dry state, the drying being effected during the ballooning of the thread.

Additional objects will become apparent from the following description, appended claims and accompanying drawings forming a part of this specification and wherein:

30 Figure 1 represents curves illustrating the shrinkage in terms of percentage residual shrinkage throughout a bobbin cake of yarn, when it is dried by the usual method and when it is dried by the process constituting this invention.

35 Figure 2 designates a schematic side elevation of a throwing machine employed in carrying out the instant process.

The foregoing objects are secured in accordance with the principles of this invention by twisting a gel yarn, i. e. a yarn that has never been dried to less than 50% moisture based on the dry weight of the yarn, and winding the twisted yarn on to a take-up device in a substantially dry or semi-dry condition. The yarn is twisted in such a manner and under such atmospheric conditions as to maintain a tension at all times at a value suitable for the requirements necessary for uniform shrinkage while the yarn is being drawn from the spin bobbin cake.

50 In the preferred embodiment of the invention, the spin bobbin cakes are washed free from acid and the yarn thrown on a standard throwing machine. In this procedure, during ballooning, the yarn is suitably dried in a convenient space so that the twisted yarn may be wound on the take-up device in a dry or semi-dry state. By 55 yarn in the "semi-dry state" is meant yarn which has never been dried to equilibrium but contains less than 50% moisture based on the dry weight of the rayon. During the unwinding and twisting of the yarn, the yarn remaining on the spin bobbin is maintained in its original gel state.

To secure the best results, I have found that there is a critical drying zone for the gel yarn, 60 wherein the yarn must be under a uniform and preferably a low tension. This critical zone may be defined as that in which the moisture content of the thread is between 1.0 times and 0.25 times the dry weight of the thread. In order 65 to secure this condition as soon as possible in the preferred embodiment of the invention, the bobbin spun cakes, after being washed to remove the acid, are centrifuged to remove the excess water and reduce the moisture content to 1.2 to 70 1.7 times the weight of the bone-dry yarn. The 75

centrifuged cake is also preferably conditioned under appropriate conditions so as to reduce the moisture content to, for example, 1.0 times, and preferably from 1.0 to 1.25 times, the weight of the bone-dry yarn. It is, of course, to be understood that it is not essential to utilize a spin bobbin cake which has been centrifuged in order to secure the benefits of the instant invention.

The final amount of moisture above equilibrium moisture which may be present in the yarn after 10 twisting can be removed in any convenient way, such as by conditioning with hot air.

In one embodiment of my invention, I subject the twisted yarn to treatment with steam or with air substantially saturated with moisture which 15 is followed by treatment with warm dry air to reduce the moisture content of the yarn to that desired.

The twisted yarn is skeined, with or without prior spooling, and the skeins subjected to the 20 desired purifying operations, i. e. bleaching and desulphuring treatments. In these treatments, the yarn shrinks substantially uniformly and the deleterious results of non-uniform shrinkage are overcome.

The purified yarn produced by the process hereinbefore described, in addition to having substantially uniform shrinkage characteristics, also is characterized by dyeing much more uniformly than the yarn of the prior art, such as yarn 30 which has been dried on the spin bobbin, twisted in the dry state, skeined and purified.

The present invention, in so far as it relates to twisting the gel thread and winding the dry or semi-dry twisted yarn, may be successfully carried out on a standard throwing machine, such as is illustrated in Figure 2 of the drawings. Referring now to Figure 2 of the drawings, wherein like reference numerals designate like parts, the reference numeral 1 designates a rigid and preferably perforated bobbin on which a cake 2 of artificial gel thread 4 produced by the viscose process has been wound. After washing free from acid and adhering bath liquors in any suitable manner, the spin bobbin 1, together with the cake 2 thereon, is positioned on a throwing spindle 3 which is operated at high speeds by any suitable and well-known means not shown in the drawings. The thread 4, as it is unwound from the revolving spin cake, balloons as indicated generally by the reference numeral 4' prior to the passage through a guide, such as a pigtail guide 5, and then passes over a glass bar 6 which adjusts the tension on the thread. During the ballooning, the yarn dries. The thread then passes on to a traversing guide 7 pivotally connected to a traversing bar 8. The traversing guide 7 directs the thread on to a take-up bobbin 9 which is rotated in any suitable manner, such as by a roll 10 which may be covered by any smooth, and preferably resilient-like material, such as gum rubber, cork or the like.

The amount of tension put into the thread, due to the ballooning, depends upon the weight of the gel thread and, therefore, its moisture content. If a soaking wet bobbin is placed on the spindle 3, that is, immediately after it has been washed without any preliminary centrifuging, the thread from the outside of the bobbin will be very heavy because it contains 200% or more water. As the 70 throwing operation continues, however, more and more water is removed from the package. Consequently, as the throwing process proceeds, the weight of the wet gel thread becomes lighter and the tension on the thread becomes less and less. 75

If the cake on the bobbin is centrifuged and conditioned prior to the throwing operation or so that the average moisture content in the gel yarn is reduced to, for example, 1.2 times the dry weight of the yarn, the tension on the thread, due to ballooning under these circumstances, will not change appreciably and the thread may be wound up at substantially constant tensions.

The pivoted traverse guide 7 in combination 10 with the glass rod 6 imparts to the thread a constant or substantially constant tension, for the angle of contact of the thread therewith does not change appreciably from the beginning to the end of the throwing operation. In place of the 15 glass rod 6, a roller (not shown) may be used. This serves to eliminate frictional tension between the thread and the guide. The roller is especially advantageous when unusually wet spin cakes are utilized.

20 It is to be understood that the expression "uniform tension" as used in conjunction with the throwing operation is not intended to define a tension which is uniform throughout the entire process. For instance, the tension on the thread 25 at the start of the throwing operation as it is wound on the take-up bobbin may possibly be 12 grams. As the process proceeds, the tension may vary as much as 1 or 2 grams from this value.

In order to more clearly explain the instant 30 invention, the following specific illustrative procedure is set forth. It is, of course, to be understood that the invention is not restricted to the precise details and procedure set forth, since they are more for illustrative purposes.

35 *Example.*—A rigid spin bobbin containing a cake of artificial thread produced from viscose by the bobbin spinning process is washed in any suitable manner, so that the spin cakes are acid-free. These spin cakes are then centrifuged to remove excess water and reduce the moisture content to 1.65 times the weight of the bone-dry yarn and allowed to condition in a room maintained at a relative humidity of 75% and a temperature of 40 75° F. which further reduces the moisture content of the cake to 1.25 to 1.0 times the weight of the bone-dry cake. This may require 20 to 30 hours. The bobbins with the spin cakes thereon are then placed on a throwing machine and thrown at a spindle speed in a range of from 3000

45 50 R. P. M. to 6000 R. P. M. in atmospheric conditions of 75% relative humidity and a temperature of 75° F. During the throwing step the yarn dries in the balloon while the spin cake retains most of its moisture. The tension on the yarn during ballooning and drying is low and uniform and, in the case of 100 denier thread, this tension may 55 vary from 6 to 14 grams, depending on the tension device and spindle speed used. The twisted yarn collected on the take-up bobbin contains 25% moisture or less. The take-up bobbin is 60 preferably perforated and of the same diameter as the spin bobbin. Following the throwing step, the twisted cake is conditioned in a suitable manner to reduce the moisture to about 6% and then 65 allowed to regain the moisture content desired for reeling. The yarn is then skeined and the skeins subjected to the purifying treatments.

An alternative method allows the omission of 70 the conditioning step but in this case, since the yarn is much heavier due to a larger amount of moisture, it is necessary to pay special attention to see that the tension on the yarn is uniform.

Still another method allows the omission of 75 the final conditioning step and permits reeling

or otherwise winding from the cake containing 25% or less of moisture.

It is to be understood that while I prefer to operate this process under the conditions of temperature and humidity above specified, in some 5 cases it may be advisable to carry out this process at higher or lower temperatures or at higher or lower humidities than herein specified. Other modifications are apparent to those skilled in the art.

10 The primary advantage of my invention is the production of a high quality thread of improved shrinkage uniformity. This is definitely shown by a comparison of the curves shown in Figure 1, wherein curve A illustrates the shrinkage characteristics of yarn produced by the bobbin spinning process and dried on the spin bobbin in accordance with the practice prior to this invention, and curve B illustrates the shrinkage characteristics of yarn produced according to the principles of the instant invention.

15 Referring to curve A, it will be noted that the yarn comprising the middle portion of the cake is shrunk to a considerably greater extent, i. e., has less residual shrinkage than either the innermost or outermost parts of the cake. This curve shows that the residual shrinkage of the yarn varies about 4% from maximum to minimum. In other words, the minimum is less than one-half the maximum.

20 Referring now to curve B, it will be noted that the difference between the maximum and minimum residual shrinkages from all parts of the spin bobbin cake is not more than 1.5%, and it is this shrinkage difference between maximum 25 and minimum residual shrinkages which I term 30 "uniform residual shrinkage".

Other advantages of my invention are improved 35 uniformity of affinity for dyes, an improved and economical process for setting the twist, improved 40 high quality yarn having few broken filaments and little fluff and improved skein formation, which enables skeins to be better dyed and otherwise treated and improves the running quality of the yarn, when the skeins are rewound. 45

Though the process has hereinbefore been described in connection with yarn by the viscose process, it is to be understood that it is applicable to the other processes of producing rayon and other synthetic fibers.

50 Since it is obvious that various changes may be made in the above description without departing from the nature or spirit thereof, this invention is not restricted thereto except as set forth in the appended claims.

55 I claim:

1. A method of producing regenerated cellulose thread having improved shrinkage characteristics which comprises removing the acid from a cake of regenerated cellulose thread wound on 60 a bobbin and which has never been dried to equilibrium, reducing the moisture in the said regenerated cellulose thread until it constitutes 1.0 to 1.7 times the weight of the dry yarn, throwing the said regenerated cellulose thread on the 65 spin bobbin at a speed that the thread during ballooning is dried to a moisture content less than 50% based on the weight of the dry thread and wound in such condition, converting into skeins and purifying.

70 75 2. A method of producing regenerated cellulose thread having improved shrinkage characteristics which comprises removing the acid from a cake of gel regenerated cellulose thread while wound on the spin bobbin, reducing the mois-

ture content of the gel regenerated cellulose thread so that it constitutes 100%-170% by weight based on the dry thread, unwinding with twisting the gel regenerated cellulose from the spin bobbin, causing the thread to travel at a speed which reduces the moisture content of said thread until it constitutes less than 50% by weight based on the dry thread, maintaining the thread under conditions permitting shrinkage, 10 winding said thread, converting into skeins and purifying.

3. In a method of producing regenerated cellulose thread having improved shrinkage characteristics, the steps which comprise washing a cake of regenerated cellulose produced by the viscose method to make said cake acid-free, reducing the moisture content of the thread until it is approximately 100 to 125% by weight based on the bone-dry thread, throwing said thread 15 at a speed that the thread during the ballooning thereof is dried to a moisture content of not more than 25% based on the weight of the bone-dry thread and wound in such condition.

4. A method of producing regenerated cellulose

thread having improved shrinkage characteristics which comprises removing the acid from a cake of regenerated cellulose wound on a bobbin and which has never been dried to equilibrium, reducing the moisture in said regenerated cellulose thread until it constitutes 1.0 to 1.7 times the weight of the dried yarn and throwing the said regenerated cellulose thread on the spin bobbin at a speed that the thread during ballooning is dried to a moisture content less than 10 5% based on the weight of the dried thread and wound in such condition.

5. In a method of producing regenerated cellulose threads having improved shrinkage characteristics, the steps comprising removing the acid from a cake of regenerated cellulose thread wound on a bobbin, reducing the moisture in the said regenerated cellulose thread until it constitutes 1.0 to 1.7 times the weight of the dry 15 yarn, twisting the said regenerated cellulose 20 thread under conditions that permit drying to a moisture content less than 50% based on the weight of the dry thread, and winding.

GEORGE SIGLER.